

## UNITED STATES PATENT OFFICE

2,169,186

## DIESEL FUEL

Bernard H. Shoemaker and Howard R. Batchelder, Hammond, Ind., assignors to Standard Oil Company, Chicago, Ill., a corporation of Indiana

No Drawing. Application June 30, 1937,  
Serial No. 151,180

8 Claims. (Cl. 44—9)

This invention relates to improvements in high speed Diesel engine fuels.

In the operation of Diesel engines in which the liquid fuel is injected directly into the cylinder, the interval between the time the fuel is injected and the time the fuel becomes ignited is called the "delay period" or ignition lag. Better engine performance is obtained when the delay period or ignition lag is of short duration since the "roughness" of running, or the Diesel knock, is directly proportional to the duration of the delay period. While it is desirable that fuels for Diesel engines in general have good ignition characteristics, it is particularly important that fuels for high speed Diesel engines have good ignition characteristics because of the extreme conditions under which they operate. The roughness of running and/or Diesel knock is most pronounced in the high speed Diesel engines, and for this reason fuels adapted for use in such engines should possess good ignition characteristics.

It is, therefore, the primary object of this invention to provide a fuel having improved ignition characteristics for high speed Diesel engines.

We have found that the ignition characteristics of high speed Diesel engine fuel oils may be materially improved by adding to such fuels 0.01% to 5%, and preferably 0.01% to 1%, of the reaction product of a mercaptan with a nitrogen oxychloride, or a nitrogen sulfochloride. These reaction products have the general formula  $RSNX_m$  and may be obtained according to the following reaction:



in which R is an alkyl or aryl group, X is sulfur and/or oxygen and m is a whole number having a value not greater than 2. The alkyl thionitrites and alkyl thionitrates may be obtained by the methods described by Rheinbold et al. in the 40 Journal für Praktische Chemie vol. 130, 133-46 (1931) and by Hans Lecher et al. in Berichte der Deutschen Chemischen Gesellschaft, vol. 59B, 1314-1321 (1926).

Specific examples of the above reaction product are:

- Butyl thionitrite  $C_4H_9SNO$
- Amyl thionitrite  $C_5H_{11}SNO$
- Amyl thionitrate  $C_5H_{11}SNO_2$
- Propyl thionitrite  $C_3H_7SNO$
- Butyl dithionitrite  $C_4H_9SNS$
- Butyl trithionitrate  $C_4H_9SNS_2$
- Benzyl thionitrite  $C_6H_5SNO$
- Benzyl dithionitrite  $C_6H_5SNS$

The term "high speed Diesel engine fuel oil" as used herein is a Diesel fuel oil having a 10% distillation point not over 460° F. and preferably not over 400° F., a 90% distillation point not over 675° F. and preferably not over 450° F. and an end distillation point not over 720° F. and preferably not over 500° F.

Having described certain specific examples of the type of compounds we may use, it is not intended that the invention be limited thereto, but it is desired to claim broadly all the inherent novelty in the invention.

We claim:

1. A high speed Diesel engine fuel comprising a fuel oil and a small amount of an organic compound having the general formula  $RSNX_m$  in which R is a radical selected from the group consisting of alkyl and aryl radicals, X is an element selected from the group consisting of oxygen and sulfur and m is a whole number having a value not greater than 2. 15

2. A high speed Diesel engine fuel comprising a fuel oil and 0.01% to 5% of an alkyl thionitrite.

3. A high speed Diesel engine fuel comprising a fuel oil and 0.01% to 5% of an aryl thionitrite. 25

4. A high speed Diesel engine fuel comprising a fuel oil having an initial distillation point not over 460° F., a 90% distillation point not over 675° F. and an end distillation point not over 720° F. and a small amount of an organic compound having the general formula  $RSNX_m$  in which R is a radical selected from the group consisting of alkyl and aryl radicals, X is an element selected from the group consisting of oxygen and sulfur and m is a whole number having a value not greater than 2. 30

5. A high speed Diesel engine fuel comprising a mineral oil having an initial boiling point less than 460° F. and an end point less than 720° F. and 0.01% to 5% of an alkyl dithionitrite. 40

6. A high speed Diesel engine fuel comprising a mineral oil having an initial boiling point less than 460° F. and an end point less than 720° F. and 0.01% to 5% of an aryl dithionitrite. 45

7. A high speed Diesel engine fuel comprising a fuel oil and 0.01% to 5% of an alkyl thionitrate.

8. A high speed Diesel engine fuel comprising a fuel oil and 0.01% to 5% of an aryl thionitrate. 50

BERNARD H. SHOEMAKER. 50  
HOWARD R. BATCHELDER.